

July 31, 1973

J. P. JONES ET AL

3,749,673

BLEACH-FABRIC SOFTENER COMPOSITIONS

Filed Feb. 22, 1971

## EFFECT OF TIME AND TEMPERATURE ON BLEACHING



## INVENTORS

John Paul Jones  
Charles H. NicolBY *John Paul Jones*  
ATTORNEY

## 1

3,749,673

**BLEACH-FABRIC SOFTENER COMPOSITIONS**  
John Paul Jones and Charles H. Nicol, Cincinnati, Ohio,  
assignors to The Procter & Gamble Company, Cincinnati, Ohio

Filed Feb. 22, 1971, Ser. No. 117,590

Int. Cl. C11d 7/54

U.S. Cl. 252—95

8 Claims

### ABSTRACT OF THE DISCLOSURE

Concentrated, dry bleach and fabric-softening compositions containing a peroxygen bleaching agent, a quaternary ammonium compound, a buffering agent and ionizable chlorine. Such compositions when dissolved in water provide fast-acting catalyzed bleaching and softening of textiles at all practical solution temperatures without the color and fabric damage usually associated with harsh hypochlorite bleaches.

### BACKGROUND OF THE INVENTION

#### (1) Field of the invention

This invention relates to dry bleach compositions having fabric softening and low color damage bleaching characteristics when employed in aqueous solution. Such compositions may also be used for cleaning sinks or dentures and for restoring natural coloring to hair after use of artificial hair coloring. As noted, these compositions are in the form of a concentrated product which can be added to water for actual use at both high and low bleaching temperatures.

The invention employs a combination of a peroxygen bleaching compound; a quaternary ammonium salt as a micelle catalyst and fabric softener; a buffering compound to maintain the bleaching solution at a proper pH and ionizable chlorine to provide a type of halogen bleaching. Preferred embodiments employ an alkali metal or alkaline earth metal chloride salt to provide at least a portion of the ionizable chlorine. Additional preferred embodiments employ a compound which will provide transition metal ions as bleaching catalysts in solution.

While acting as micelle catalysts for the bleaching reaction, the quaternary ammonium salts retain their fabric softening capabilities and can also provide a source of necessary chloride ions. The non-quaternary chloride compounds (e.g., alkali metal or alkaline earth metal chlorides) must be employed in the present compositions to provide chloride ions if the quaternary ammonium compound does not provide these ions in sufficient concentration. Inclusion in the instant dry compositions of a source of transition metal ions is not essential to the invention but enhanced bleaching performance is obtained if such a source compound is employed.

#### (2) Description of the prior art

Several types of bleaching compositions for home use are known in the art. A commonly encountered household bleach is in the form of a liquid solution employing a hypochlorite species as the bleaching active. Such compounds are effective stain-removing bleaches when used in relatively high concentrations, but these hypochlorite or active chlorine bleaches also cause rather severe damage to fabric colors and can in addition damage textile fibers with repeated use. Liquid bleaches of this type also pre-

## 2

sent handling and packaging problems. While color and fabric damage may be minimized by employing milder oxygen bleaches such as potassium monopersulfate, soil and stain removal characteristics of these oxygen bleaches are much less desirable than those of the halogen bleaching agents.

Likewise, several types of fabric softeners are presently available for home use, but all must be added separately to the fabric rinse solution since they are chemically incompatible with many laundering products.

Many of the above-described shortcomings of prior art compositions are overcome by a chlorine-free bleaching composition described in the concurrently filed application of John Paul Jones and Charles H. Nicol entitled "Bleach Compositions," Ser. No. 117,814, filed Feb. 22, 1971. It is an object of the present invention to provide an improved concentrated chlorine-containing bleaching composition which can be safely applied to colored as well as white fabrics. It is a further object of this invention to provide a compatible bleach-fabric softener combination which is utilized in the form of a single, easily handled, dry composition. It is a further object of the present invention to provide a catalyzed bleach-fabric softener composition which can be employed at low solution concentration and which is effective at low temperatures and after short fabric contact time.

While bleach and fabric softening compositions containing certain of the above-mentioned components have been disclosed in the prior art, it has now been discovered that by combining certain types of catalysts with the designated bleaching agents, a combined bleaching and fabric softening product can be created which accomplishes the above objectives and which is unexpectedly superior to that attainable using the compositions of the prior art.

### SUMMARY OF THE INVENTION

Dry, concentrated, bleach-fabric softener compositions and methods for using said compositions are provided. The compositions consist essentially of:

(a) about 8% to 60% by weight of a peroxy bleaching agent selected from the group consisting of sodium or potassium monopersulfate; organic peroxy acids (or water-soluble salts thereof) of the general formula



wherein R is a substituted or unsubstituted alkylene or arylene group and Y is



or any other group which in water yields an anionic group; and mixtures thereof;

(b) about 10% to 60% of a quaternary ammonium compound of the general formula



or



wherein  $R_1$  is an alkyl group containing from about 12 to 20 carbon atoms,  $R_2$  is selected from the group consisting of alkyl groups containing about 1 to 14 carbon atoms, cycloalkyl groups containing about 5 to 8 carbon atoms, carboxymethyl groups, aryl groups containing from 6 to 8 carbon atoms, alkaryl groups containing from 7 to 10 carbon atoms, pyridyl and groups of the general formula  $-(C_3H_6O)_a(C_2H_4O)_bH$  wherein  $a$  and  $b$  are integers and  $a+b$  is 1 to 50;  $R_3$ ,  $R_4$  and  $R_5$  are each selected from the group consisting of alkyl groups containing about 1 to 3 carbon atoms, cycloalkyl groups containing about 5 to 8 carbon atoms, carboxymethyl groups, aryl groups containing from 6 to 8 carbon atoms, alkaryl groups containing from about 7 to 10 carbon atoms, pyridyl, and groups of the general formula  $-(C_3H_6O)_a(C_2H_4O)_bH$  wherein  $a$  and  $b$  are integers and  $a+b$  is 1 to 50;  $R_6$  is a group within the definition of the  $R_3$ ,  $R_4$  and  $R_5$  groups or H;  $R_7$  is an alkylene group containing from 1 to 3 carbon atoms, an arylene group containing from 5 to 8 carbon atoms or a group having the formula



$X$  is chloride, fluoride, nitrate, sulfate, methylsulfate, carbonate, hydrogen phosphate, dihydrogen phosphate, chlorate or hydroxide; and  $n$  is 1 when  $X$  is monovalent and  $n$  is 2 when  $X$  is divalent;

(c) about 10% to 75% by weight of a buffering agent effective to maintain the pH of said compositions in aqueous solutions within the range of from 7 to 10; said compositions containing from about 5 to about 100 grams of ionizable chlorine per kilogram of the total composition. The compositions can contain from about 1% to 15% by weight of an alkali metal or alkaline earth metal chloride to provide all or part of the ionizable chlorine. Alternatively, all of the ionizable chlorine can be provided by the quaternary ammonium compound as hereinafter detailed. A preferred embodiment of the invention contains, in addition to the above components, from about 0.08% to about 8% by weight of a water-soluble salt of a transition metal element.

The compositions are dissolved in water to provide fabric softening and catalyzed bleaching of both colored and white fabrics. Such aqueous solutions may also be used as hard surface or denture cleaners and as agents for restoring natural color to artificially colored hair.

#### BRIEF DESCRIPTION OF THE DRAWING

The drawing provides a graphical representation of the effect of time and temperature upon the bleaching activity of the compositions of the instant invention relative to the prior art. The horizontal axis represents time in minutes. The vertical axis represents  $\Delta W$ , a measure of stain removal performance described in column 9, lines 73-75, hereof. Each curve represents a particular bleaching composition of Table I (col. 9) identified by number and utilized at the indicated temperature.

#### DETAILED DESCRIPTION OF THE INVENTION

At this juncture the theoretical nature of the present catalyzed bleaching system and the individual components of the compositions will be described in detail.

##### (A) Catalysis of bleaching reactions

Although the scope of the present invention is not limited by any particular theory, the monopersulfate bleaches of this invention are believed to ionize in the bleaching solution according to the equation



The  $\text{HSO}_5^-$  further dissociates in solution as follows:



It has been discovered that the effectiveness of the persulfate bleaching is dependent on the formation in solu-

tion of a bi-anionic transition state complex having the formula



Such a complex is formed from the  $\text{SO}_5^=$  and  $\text{HSO}_5^-$  anions present in the bleaching solution.

The organic mono- and diperoxyacid bleaches of the instant compositions, representative compounds having the general formulas,



wherein R is an alkylene or arylene group, likewise form bi-anionic dimers during the bleaching process. As with the monopersulfates, such complexes are formed from the combination of (1) the above compounds which have lost one proton upon dissolution and/or (2) the above compounds which have lost both protons. Thus, these bi-anionic complexes, for example, can have the general formulas,



or if the above two representative compounds are mixed,



or



wherein R is again an alkylene or arylene group.

It has been discovered that formation of these various complexes from two negatively charged ions can be facilitated by the addition to the solution of positively charged micelles and/or transition metal ions.

A micelle is a highly charged colloidal aggregate. It is believed that such positively charged aggregates, as well as positive transition metal ions, serve as rallying points for the  $\text{SO}_5^=$  and  $\text{HSO}_5^-$  anions and their organic peroxy-acid counterparts, thereby facilitating formation of the indispensable transition complex of the bleaching reaction. Quaternary ammonium salts are employed in order to form the necessary micelles in solution. In addition, bleaching catalysis may be enhanced by addition of a transition metal salt such as copper sulfate, to provide more complex-creating cations in solution.

Bleaching activity is enhanced even further by virtue of chloride ions in bleaching solutions. Consequently, dry compositions of the present invention must contain enough of a water-soluble chloride compound or mixtures thereof to provide from about 5 to about 100 grams of ionizable chlorine per kilogram of dry composition. Ionizable chlorine is that portion of any compound of the present invention which when dissolved contributes chloride ions to the aqueous solutions. Ionizable chlorine is, of course, provided by chloride salts. The necessary ionizable chlorine content of the instant composition can be provided in the form of the quaternary ammonium chloride, an added alkali metal or alkaline earth metal chloride and/or by the transition metal chlorides. It is known that these chloride salts in solution with certain oxygen bleaches do not yield chloride ions but rather, in combination with such oxygen bleaches, provide enhanced bleaching of a hypochlorite type. It has been discovered, however, that addition of chloride ions to a micelle-catalyzed oxygen bleaching system yields an active chlorine species in solution to provide mixed oxygen-chlorine bleaching even more effective than the known hypochlorite-forming peroxygen/chloride salt combination. Furthermore, this effective bleaching is accomplished at a much lower composition concentration in

solution than prior art hypochlorite-forming combinations.

It is believed that the effective micelle catalysis of the bleaching reaction is responsible for the very favorable color damage characteristics of the instant compositions. Although some hypochlorite is formed in solution from the compositions of the instant invention, it is formed over an extended period of time and at a lower concentration than the directly added hypochlorite of the prior art. Performance "loss" due to this indirect method of hypochlorite bleaching is more than adequately compensated for by the effectiveness of the micelle-catalyzed oxygen bleaching. Overall bleaching performance thus compares favorably with harsh concentrated hypochlorite with little hypochlorite-type color damage occurring.

It should be noted that the compositions of the instant invention should contain no more bromide than would be present if the optional transition metal salt is a bromide. This is so since large amounts of bromide ions in solution with some peroxygen bleaches can cause severe color damage to fabrics. Consequently, the quaternary ammonium compound (which can be present in a relatively high concentration in the composition) cannot be a bromide salt, i.e. bromide is an "interfering" anion.

#### (B) Individual components

(1) Bleaching agents.—The principal bleaching actives in the instant compositions are sodium or potassium monopersulfate ( $\text{NaHSO}_5$  and  $\text{KHSO}_5$ ) and the organic mono- and diperoxyacids (or water-soluble salts thereof) having respectively the following formulas:



and



wherein R can be alkylene or arylene and Y can be any group which yields an anionic moiety in solution such as



Potassium monopersulfate is available commercially from E. I. du Pont de Nemours and Company under the trade name "Oxone." It contains approximately 42.8% by weight  $\text{KHSO}_5$ , the balance being  $\text{KHSO}_4$  and  $\text{K}_2\text{SO}_4$  in about equal proportions.

The organic peroxyacids or salts thereof of the invention, as noted above, can contain either one or two peroxy groups and can be either aliphatic or aromatic. When the organic peroxyacid is aliphatic, the unsubstituted acid has the general formula



where Y, for example, can be



and n can be an integer from 1 to 12 with perazelaic acids (n=7) being the preferred compounds. The alkylene linkage between the anionic groups can contain halogen or other non-interfering groups.

When the organic peroxyacid is aromatic, the unsubstituted acid has the general formula



Where Y is



for example. The



and YH groupings can be in any relative position around the aromatic ring. The ring can contain any noninterfering substituent such as halogen groups. Examples of suitable aromatic peroxy acids include monoperoxyphthalic acid, diperoxyterephthalic acid, 4-chlorodiperoxyphthalic acid and the monosodium salt of diperoxyterephthalic acid. The preferred aromatic peroxyacids are the mono- and diperoxyisophthalic acids.

The bleaching compositions can contain from about 8% to about 60% by weight of the bleaching agent. The preferred monopersulfate weight range is from about 25% to about 30% by weight. A preferred organic peroxyacid weight range is from about 16% to about 35% by weight. Mixtures of the monopersulfate compounds and the peroxyacids can be employed in the instant invention.

These bleaching compositions are, of course, dissolved in aqueous solutions for actual use on fabrics, sinks, dentures or hair. Depending upon the bleaching strength desired and the intended use, the bleaching composition is added in quantities sufficient to yield from about 5 to 80 p.p.m. available oxygen in solution from either the persulfate or organic peroxyacid bleach actives. The above bleaching actives when employed in the catalyzed compositions of the present invention provide effective bleaching at all practical bleaching solution temperatures and bleach effectively after a very short contact time with the material to be bleached. As noted, color and fabric damage is minimal.

(2) Quaternary ammonium compounds.—Quaternary ammonium compounds useful herein have the general formulas



and



wherein  $\text{R}_1$  is an alkyl group containing from about 12 to 20 carbon atoms,  $\text{R}_2$  is an alkyl group of about 1 to 14 carbon atoms, a cycloalkyl group of about 5 to 8 carbon atoms, a carboxymethyl group, a 6 to 8 carbon aryl group, an alkaryl group of 7 to 10 carbon atoms, a pyridyl group, or a group of the general formula



wherein  $a$  and  $b$  are integers and  $a+b$  is 1 to 50;  $\text{R}_3$ ,  $\text{R}_4$  and  $\text{R}_5$  are either alkyl groups of about 1 to 3 carbon atoms, cycloalkyl groups of about 5 to 8 carbon atoms, carboxymethyl groups, 6 to 8 carbon aryl groups, alkaryl groups of 7 to 10 carbon atoms, pyridyl groups, or groups of the general formula  $-(\text{C}_3\text{H}_6\text{O})_a(\text{C}_2\text{H}_4\text{O})_b\text{H}$  wherein  $a$  and  $b$  are integers and  $a+b$  is 1 to 50;  $\text{R}_6$  falls within the definition of the  $\text{R}_3$ ,  $\text{R}_4$  or  $\text{R}_5$  groups or is H;  $\text{R}_7$  is

either a 1 to 3 carbon atom alkylene group, a 5 to 8 carbon arylene group or a group of the formula



X is any non-interfering anion such as chloride, nitrate, fluoride, sulfate, methylsulfate, carbonate, hydrogen phosphate, dihydrogen phosphate, chlorate or hydroxide; and n is 1 when X is monovalent and n is 2 when X is divalent. Examples of quaternary ammonium compounds employable in the compositions include tetradecltrimethylammonium chloride; tetradecltrimethylammonium methylsulfate; tetradecltrimethylammonium nitrate; cetyltrimethylammonium hydrogen phosphate;



cetyltrimethylammonium nitrate; octadecyltrimethylammonium chloride; octadecyltrimethylammonium chlorate; octadecyltrimethylammonium nitrate; eicosyltrimethylammonium chloride; eicosyltrimethylammonium hydroxide; eicosyltrimethylammonium nitrate;



$[\text{C}_{20}\text{H}_{39}\text{N}(\text{CH}_3)_3]_2\text{HPO}_4$ , the alkyl dimethyl ethylbenzyl ammonium chlorides of Petrocci et al., U.S. Pat. 3,525,793, Aug. 25, 1970; Armour Industrial Chemical Company's "Ethoquad" and "Propoquad" and singly or doubly quaternized compounds derived from Wyandotte Chemical Corporation's "Tetronic" compounds. Preferred quaternary ammonium compounds are the  $\text{C}_{16}$ ,  $\text{C}_{18}$  and  $\text{C}_{20}$  alkyltrimethylammonium chlorides. Depending upon the particular quaternary ammonium compound employed, the compositions contain from about 10% to about 60% by weight of the quaternary ammonium component.

The quaternary ammonium constituent serves two purposes in the instant compositions. These surface active compounds form the micelles for catalysis of the per-oxygen bleaching, and in addition they impart fabric softening characteristics to the bleaching solutions. In solutions prepared from the compositions of this invention the quaternary ammonium salt concentration should range from about 100 p.p.m. to about 500 p.p.m.

It is well-known that quaternary ammonium compounds of the type herein employed function as fabric softeners. They have heretofore been utilized alone in laundry rinse water since they are incompatible with anionic detergents. It has been discovered, however, that these compounds are compatible with the biamionic, complex-forming bleach agents of the present invention and, in fact, act as micelle catalysts while retaining their fabric softening properties.

It has been found that the shorter chain quaternary ammonium salts ( $\text{C}_{14-18}$ ) provide slightly better micelle catalysis while the longer chain salts  $\text{C}_{18-20}$  are better fabric softeners. Consequently, a mixture of long and short chain quaternary ammonium compounds is preferred for use in the instant compositions. Thus a preferred embodiment of the invention is a dry composition which contains about 2% to about 30% by weight of a 20 carbon chain quaternary ammonium salt and about 8% to 30% by weight of 14, 16 or 18 carbon chain quaternary ammonium salts. In aqueous solution prepared from this preferred composition there should be from about 20 p.p.m. to about 80 p.p.m. of the  $\text{C}_{18-20}$  quaternary ammonium salt to provide softening capability. As discussed more fully below, the quaternary ammonium compound, if a chloride salt, can contribute to the total required ionizable chlorine content of the composition.

(3) Buffering agent.—It has been discovered that micelle catalysis and formation of the biamionic complexes discussed above are greatly facilitated by maintenance of the bleaching solution at a carefully controlled pH. The pH of the solution at which the concentration of the  $\text{SO}_5^{2-}$  and  $\text{HSO}_4^-$  anions are equal (the  $\text{pK}_a$ ) occurs at a pH of 9.2. The  $\text{pK}_a$  of the organic peroxyacid system is from a pH of 7 to 8. Consequently the best bleaching

performance occurs when the pH of the bleaching solution is maintained between about 7 and about 10. Outside this pH range, bleaching performance diminishes markedly.

To maintain this controlled pH in solution, any non-interfering compound which can alter and maintain pH such as any standard buffering agent or combination is employed. For example, phosphates, carbonates or bicarbonates which buffer within the 7-10 pH range are useful. Examples of suitable buffering agents include sodium bicarbonate, sodium carbonate, disodium hydrogen phosphate and sodium dihydrogen phosphate. Sodium carbonate is the preferred buffering agent for monopersulfate systems. Disodium hydrogen phosphate and sodium dihydrogen phosphate are preferred for peroxy acid systems. Other buffering compositions for any desired pH can be obtained by the skilled artisan from any standard chemistry handbook or textbook. Buffering agents comprise from about 10% to about 75% by weight of the compositions.

(4) Alkali metal or alkaline earth metal chloride.—Addition of a compound of this type to the concentrated bleaching composition of this invention is optional if the quaternary ammonium compound is a chloride and is present in the dry compositions in sufficient amount to provide the necessary 5 to 100 grams of ionizable chlorine per kilogram of the total composition. If, however, the quaternary ammonium compound is not a chloride or is not present in an amount sufficient to provide the proper ionizable chlorine content, this alkali metal or alkaline earth metal chloride is a necessary component. Suitable chlorides include, for example,  $\text{NaCl}$ ,  $\text{KCl}$ ,  $\text{CaCl}_2$  and  $\text{MgCl}_2$ .

When the alkali metal or alkaline earth metal chloride is employed, it should comprise from about 1% to 15% by weight of the total composition. In general, preferred embodiments of the present invention employ enough chloride compound of any type so that in solution the chloride ion (although as noted above, the chloride ion as such probably does not exist in the bleaching solution) is present from whatever source in a theoretical p.p.m. amount equal to the p.p.m. of available oxygen (av.  $\text{O}_2$ ) from the oxygen bleaching actives. A more specific preferred embodiment of the present invention would employ a quaternary ammonium chloride of the type defined above in an amount of from about 15% to about 25% by weight with an alkali metal or alkaline earth metal chloride compound being present in a concentration of from about 2% to about 10% by weight.

(5) Transition metal salt.—Improved bleaching can also be obtained by the optional addition to the compositions of a source of transition metal ions. Any soluble salts which yield such ions in bleaching solution are useful in this invention. Such ions are believed to further catalyze the formation of the active peroxy compound and chlorine species to provide synergistic bleaching enhancement.

Transition metal salts which can be used in the instant compositions include copper sulfate, copper chloride, cobalt chloride, manganese bromide, nickel nitrate, copper nitrate, chromium chloride, manganese nitrate and chromium bromide. It should be noted that if chloride transition metal salts are employed, they also can contribute to the necessary ionizable chlorine content of the compositions.

Such transition metal salts can be employed in the present compositions in a concentration range of from about 0.08% to about 8% by weight. The salts are preferably present in an amount effective to provide a transition metal ion concentration in bleaching solution of from about  $5 \times 10^{-6}$  M to about  $3 \times 10^{-5}$  M.

(6) Other additives.—Other optional additives such as builders, perfumes, coloring agents, fillers, etc., can be added to the dry bleaching and softening compositions. These additional components, however, must not interfere

with the essential chemical or physical functioning of the compositions as catalyzed bleaches and fabric softeners.

The above-described components of the bleaching compositions of this invention are all available in dry form. Formulation, therefore, of dry compositions is simply accomplished by thoroughly mixing the granular or powdered components together in the appropriate weight percentage concentrations. It would be possible to provide a bleaching solution containing the components of this present invention by adding such components to the bleaching solution in liquid form. Besides creating handling and packaging problems, however, concentrated liquid compositions of this type are relatively unstable and tend to rapidly degrade upon standing.

Despite the powerful bleaching activity of the micelle-catalyzed, oxygen-chlorine agents herein, textile fiber damage is comparable to perborate washing agents. In addition, the bleaching solution resulting from the compositions of the present invention do not cause running of textile colors or undesirable color transfer. The fast-acting low temperature bleaching activity of the dissolved compositions makes the present invention especially suited for use in fabric rinse water after normal textile laundering.

The following tests serve to illustrate the bleaching, softening and other performance properties of the compositions of the instant invention. Table I provides 16 concentrated bleaching compositions by component weight percentages. Compositions Nos. 2, 3, 4, 5, 6, 9, 10, 12 and 15 are representative examples of compositions of the instant invention. Composition No. 8 contains dihydrogenated tallow ammonium monoperoxyulfate. Composition No. 11 is a hypochlorite formulation. Composition No. 16 is a potassium dichloroisocyanurate composition. The others are compositions with one or more of the essential components of the instant invention omitted. These compositions are employed in the following Bleaching Performance Test, Color Damage Test, Bleaching Time and Temperature Test, and Fabric Softening Test.

TABLE I

| Concentrated composition number.....                 | 1    | 2  | 3    | 4  | 5    | 6  | 7  | 8  | 9     | 10    | 11   | 12 | 13   | 14   | 15 | 16   |
|------------------------------------------------------|------|----|------|----|------|----|----|----|-------|-------|------|----|------|------|----|------|
| Component, weight percent:                           |      |    |      |    |      |    |    |    |       |       |      |    |      |      |    |      |
| Potassium monopersulfate.....                        | 27   | 25 | 23   | 27 | 29   | 25 | 25 | 25 | 25    | 25    | 27   | 31 | 18   | 25   | 25 | 25   |
| Diperazelaic acid.....                               |      |    | 24   |    |      |    |    |    |       |       |      |    |      |      |    |      |
| Monoperoxyphthalic acid.....                         |      |    |      |    |      | 25 |    |    |       |       |      |    |      |      |    |      |
| Diperoxyisophthalic acid.....                        |      |    |      |    |      |    |    |    |       |       |      |    |      |      |    |      |
| Dihydrogenated tallow ammonium monoperoxyulfate..... |      |    |      |    |      |    |    |    | 10    |       |      |    |      |      |    |      |
| Sodium hypochlorite.....                             |      |    |      |    |      |    |    |    | 85    |       |      |    |      |      |    |      |
| Potassium dichloroisocyanurate.....                  |      |    |      |    |      |    |    |    |       |       |      |    |      |      |    | 5.25 |
| Elcosyltrimethylammonium chloride.....               |      |    | 7    |    |      | 3  |    | 3  | 3     |       | 3    |    | 3    |      |    | 15   |
| Octadecyltrimethylammonium chloride.....             |      | 28 |      |    |      | 12 |    |    |       |       |      | 12 |      |      |    |      |
| Cetyltrimethylammonium choride.....                  |      |    | 12   |    |      |    |    |    |       |       |      |    | 12   |      |    |      |
| Ethoquad 18/12 <sup>1</sup> .....                    |      |    |      | 27 |      |    |    |    |       |       |      |    |      |      |    |      |
| Cetyltrimethylammonium nitrate.....                  | 14   |    |      |    | 25   |    |    | 38 |       |       |      |    |      |      |    |      |
| Sodium choride.....                                  | 6    |    |      |    | 15   |    | 7  | 10 |       | 6     |      | 42 | 6    |      |    |      |
| Chloride ion content (g. Cl-/kg. composition).....   | 16.8 | 35 | 22.4 | 90 | 15.5 | 7  | 10 | 63 | 19.5  | 18.5  | 15.5 | 42 | 19.5 |      |    |      |
| Copper sulfate.....                                  |      |    |      |    |      |    |    |    |       |       |      | .2 |      |      |    |      |
| Buffer*.....                                         | 22   | 21 | 12   | 20 | 20   | 22 | 24 | 15 | 26    | 18    | 20   | 22 | 26   | 15   | .2 |      |
| Inerts.....                                          | 37   | 36 | 29   | 30 | 15   | 38 | 40 | 13 | 33.82 | 94.75 | 35.8 | 43 | 25   | 33.8 | 85 |      |

<sup>1</sup> See the following formula—



The Bleaching Performance Test analyzes bleaching performance of the various compositions of Table I. A Tergotometer (United States Testing Company) operated at a constant agitation rate of 80 c.p.m. is used for all experiments. Unless otherwise stated, runs are made at 120° F. for 10 minutes. Swatches are graded before and after bleaching on a Hunter Color Difference Meter. An initial and final whiteness grade was calculated from the Hunter color coordinates (L, a, b) for each swatch through the use of the whiteness equation

$$W = 100 - \sqrt{(100 - L)^2 + a^2 + b^2}$$

and the color differences,  $\Delta W$ , so obtained were taken as a measure of stain removal performance. The average  $\Delta W$  values for five stains are reported in the example

65

75

(grass, tea, wine, gravy and Empa-Sulfur Black). A  $\Delta W$  difference of 2 is readily apparent to the human eye.

#### PREPARATION OF STAINED SWATCHES

5 The swatches used in the development of these tests are obtained from several sources. The respective swatches and their sources (commercial or method of preparation) are outlined in the following summary.

##### Grass stain

10 200 g. of freshly cut untreated grass is mixed with 1000 cc. of 5 gr./gal. hardness water in a Waring Blender until a uniform slurry is produced. This slurry is strained through cotton, and the resulting extract is used in the Atlas Electric Padder by passing the cloth through three successive times. The cloth is aged three days and stored in the dark.

##### Tea

25 20 ounces of Lipton tea is added to 1½ gallons of 5 gr./gal. hardness water and simmer-boiled for 2 hours. The solution is filtered through cotton cloth and liquor made up to 1½ gallon with hot water. Two square yards of cotton are immersed into the 3% tea solution. The temperature is raised to boil and maintained for two hours. The cloth is lifted out of the liquor and transferred to about 3 gallons of 5 gr./gal. water (pH=9.5) at 100° F. to rinse. Wringing is done using the Atlas Electric Padder. The cloth is ironed to fix the stain and allowed to age for three days at 120° F.

##### Gravy

30 35 A one ounce package of Durkee's brown gravy mix is mixed with 1 cup of water and brought to a boil with stirring. The mixture is removed from the heat and stirred with a high-shear homogenizer for 5 minutes. The warm gravy solution is then placed in a container and the cloth

wherein R is stearyl and the compound contains 2 moles combined ethylene oxide and has a molecular weight of 422. See Armour Industrial Chemical Company Technical Bulletin F-4.

\*For Compositions 1, 2, 4, 6, 7, 8, 10, 12, 13, 14 and 15 the buffering agent is sodium carbonate. For Compositions 2, 5 and 9 the buffering agent is a mixture of disodium hydrogen phosphate and sodium dihydrogen phosphate in a Na<sub>2</sub>HPO<sub>4</sub> to NaH<sub>2</sub>PO<sub>4</sub> ratio of approximately 5:1.

is run through the solution and padded. The stained cloth is then dried in an oven. Two applications are given.

##### Empa-sulfur black and red wine

These cloth samples are obtained commercially from Test Fabrics Inc., 55 Vandam St., New York 13, N.Y., manufactured by E.M.P.A., Unterstasse II, 9001 St. Gall, Switzerland.

#### BLEACHING PERFORMANCE TEST

70 Bleaching activity of Compositions of Table I is compared. Table II provides the concentration in bleaching solution of components of the various compositions. Table II also summarizes the  $\Delta W$  value of each composition, thereby indicating their relative bleaching performance.

TABLE II

| Concentrated composition number                              | 1    | 2    | 3*  | 4    | 6*   | 7   | 8   | 10   | 11   | 11* | 12*  | 13 | 14  | 15*   | 16*       |
|--------------------------------------------------------------|------|------|-----|------|------|-----|-----|------|------|-----|------|----|-----|-------|-----------|
| Component—solution concentration:                            |      |      |     |      |      |     |     |      |      |     |      |    |     |       |           |
| Potassium monopersulfate (p.p.m. av. O <sub>2</sub> )        | 45   | 45   | —   | 45   | 44   | 45  | —   | 45   | —    | —   | 44   | 45 | 45  | 44    | —         |
| Diperoxazelaic acid (p.p.m. av. O <sub>2</sub> )             | —    | —    | 25  | —    | —    | —   | —   | —    | —    | —   | —    | —  | —   | —     | —         |
| Dihydrogenated tallow ammonium monoperoxy-                   | —    | —    | —   | —    | —    | —   | 37  | —    | —    | —   | —    | —  | —   | —     | —         |
| sulfate (p.p.m. av. O <sub>2</sub> )                         | —    | —    | —   | —    | —    | —   | —   | 44   | 200  | 200 | —    | —  | —   | —     | —         |
| Sodium hypochlorite (p.p.m. av. Cl <sub>2</sub> )            | —    | —    | —   | —    | —    | —   | —   | —    | —    | —   | —    | —  | —   | —     | —         |
| Potassium dichloroisocyanurate (p.p.m. av. Cl <sub>2</sub> ) | —    | —    | —   | —    | —    | —   | —   | —    | —    | —   | —    | —  | —   | —     | 120       |
| Eicosyltrimethylammonium chloride (p.p.m.)                   | 50   | —    | —   | 50   | —    | —   | —   | 50   | —    | —   | 50   | —  | —   | 50    | —         |
| Octadecyltrimethylammonium chloride (p.p.m.)                 | 203  | —    | —   | 200  | —    | —   | —   | —    | —    | —   | 200  | —  | —   | 200   | —         |
| Cetyltrimethylammonium chloride (p.p.m.)                     | 200  | —    | —   | —    | —    | —   | —   | 200  | —    | —   | —    | —  | —   | —     | —         |
| Ethoquad 18/12 <sup>1</sup> (p.p.m.)                         | —    | —    | —   | 500  | —    | —   | —   | —    | —    | —   | —    | —  | —   | —     | —         |
| Cetyltrimethylammonium nitrate (p.p.m.)                      | 230  | —    | —   | —    | —    | —   | —   | —    | —    | —   | —    | —  | —   | —     | —         |
| Sodium chloride (p.p.m.)                                     | 100  | —    | —   | 100  | —    | —   | —   | 100  | —    | —   | —    | —  | —   | 1,000 | 100       |
| Copper sulfate (M×10 <sup>-4</sup> )                         | —    | —    | —   | —    | —    | —   | —   | 1    | —    | —   | 1    | —  | —   | 1     | —         |
| Initial Solution pH                                          | 9.3  | 7.5  | 9.5 | 9.0  | 9.5  | 9.3 | —   | —    | —    | —   | 9.0  | —  | —   | 9.0   | —         |
| ΔW                                                           | 10.0 | 12.3 | 16  | 10.3 | 12.3 | 4.8 | 2.5 | 17.2 | 10.8 | 20  | 20.7 | 12 | 6.4 | 6.3   | 13.3 17.5 |
| Color damage index                                           | 8    | —    | 5   | —    | —    | —   | —   | 28   | —    | 6   | —    | —  | —   | 14    | 16        |

<sup>1</sup> See Table I, footnote 1.

\*These compositions were used after or as the cloths were washed in "Tide" at 125° F. with 7 grain/gallon hardness water.

It can be seen from Table II that the compositions of the instant invention provide stain removal superior to the other prior art compositions at comparable strength in solution and superior to compositions not containing all of the essential components of the instant invention. Preferred Composition No. 10 performs at a very low strength about as well as a highly concentrated NaOCl bleaching solution (No. 11). Substantially similar ΔW results are obtained with the compositions of the present invention not appearing in Table II (Nos. 5 and 9).

When the potassium monopersulfate of Compositions 2, 4, 6, 10, 12 and 15 is replaced with sodium monopersulfate and when the diperazelaic acid of Composition 3 is replaced with monoperazelaic acid, substantially similar performance results are obtained.

When the diperoxyisophthalic acid of Composition 9 is replaced with diperoxyterephthalic acid, 4-chlorodiperoxyphthalic acid, the monosodium salt of diperoxy-

monium fluoride, sulfate, methylsulfate, hydrogen phosphate, dihydrogen phosphate, chlorate, carbonate or hydroxide substantially similar performance of the compositions is obtained.

#### COLOR DAMAGE TEST

Color damage characteristics of the compositions of the instant invention are compared to each other and to the other compositions of Table I. Color damage is ascertained and evaluated by the following procedures. Thirty-two different articles of clothing having characteristics summarized in Table III are first washed in "Tide," a representative commercially available laundering detergent, with water of 7 grain hardness at 125° F. Compositions 11 and 16 were employed in the wash water itself. The other compositions were utilized in 7 grain hardness rinse water at 100° F. All compositions were employed at the concentrations of Table II.

TABLE III.—CLOTHING USED FOR COLOR DAMAGE TEST

| Fiber content            | Color               | Item            | Brand                    |
|--------------------------|---------------------|-----------------|--------------------------|
| Cotton                   | Yellow              | Girl's dress    | Bonnie Press.            |
| Do                       | Blue                | Sheet           | Wamsutta Lustercare.     |
| Do                       | Turquoise           | Towel           | Stevens Utica.           |
| Do                       | Green               | Girl's dress    | Bonnie Press.            |
| Do                       | Black               | Man's slacks    | Wrangler.                |
| 50% polyester/50% cotton | Turquoise           | Child's shirt   | True Merit.              |
| Do                       | do                  | Woman's skirt   | Donnkenny.               |
| Polyester                | Yellow              | Woman's shell   | Sweetree.                |
| Do                       | Red                 | Woman's dress   | John Meyer.              |
| Do                       | Blue                | Woman's slacks  | S.S. Kresge.             |
| Do                       | Black               | do              | Do.                      |
| Acetate                  | Yellow              | Woman's shell   | W.T. Grant Co.           |
| Do                       | Blue                | Woman's dress   | Berkshire B-Tween.       |
| Do                       | Black               | Woman's shell   | W.T. Grant Co.           |
| 85% arnel/15% nylon      | Yellow              | Woman's dress   | Jule-Wyn.                |
| 95% arnel/5% nylon       | Blue                | do              | Hargro.                  |
| Do                       | Black               | Man's shirt     | McGregor Miracle.        |
| Orlon acrylic            | Pink                | Woman's sweater | Talbot Taralan.          |
| Acrylic                  | Green               | Boy's shirt     | Garan.                   |
| Anton nylon              | Yellow              | Woman's slip    | Vassarette.              |
| Do                       | Blue                | do              | Do.                      |
| Nylon                    | Red                 | do              | S.S. Kresge.             |
| Do                       | Black               | Woman's shell   | Cobble Knits.            |
| Wool                     | Yellow              | Man's vest      | McGregor Scotch & Water. |
| Do                       | Blue                | Man's sweater   | Alan Paine.              |
| Creslan acrylic          | Aqua                | Girl's skirt    | Aileen.                  |
| 75% cotton/25% nylon     | Blue                | Girl's slacks   | Do.                      |
| Cotton                   | Yellow              | Woman's slacks  | Do.                      |
| Do                       | Yellow/white stripe | Woman's blouse  | Do.                      |
| Creslan acrylic          | Green               | Woman's slacks  | Do.                      |
| DuPont nylon             | White               | Fabric          | Warner.                  |
| Nylon                    | do                  | Woman's slip    | Warner.                  |

terephthalic acid or a monoperoxy compound of the general formula



wherein R is an alkyl group of from about 8 to about 18 carbon atoms and wherein X<sup>1</sup> and Y<sup>1</sup> are each selected from the group of cations consisting of hydrogen, sodium, potassium, ammonium and substituted ammonium cations, substantially similar performance results are obtained.

When the cetyltrimethylammonium nitrate of Compositions 4 and 9 is replaced with cetyltrimethylammonium

After only two cycles (many fewer than the number of times an article of clothing would be bleached in the home over a period of time) each article was graded on a scale from 0 to 3. 0 corresponded to no color change; 1 to slight change; 2 to noticeable change and 3 to damage leaving the article unwearable. The value grades from all 32 articles were then added to provide a composite color damage indication for each composition tested.

Each composition tested for color damage was also tested for bleaching performance in a manner similar to that used in the Bleaching Performance Test. ΔW values after one cycle were ascertained as in the Bleaching Performance Test. It should be noted that the ΔW values

of those compositions tested for fabric damage (marked with asterisks in Table II) also include stain removal from the Tide wash as well as bleaching of the tested compositions.

Color damage indices and  $\Delta W$  values are summarized in Table II. It is readily apparent that compositions of the present invention provide relatively high  $\Delta W$  values at relatively low color damage levels.

#### BLEACHING TIME AND TEMPERATURE TEST

Composition Nos. 10, 11 and 13 of Table I are placed in bleaching solutions in the component concentrations described in Table IV.

TABLE IV

| Concentrated composition number                       | 10  | 11 | 13 |
|-------------------------------------------------------|-----|----|----|
| Component—solution concentration, p.p.m.:             |     |    |    |
| Potassium monopersulfate (p.p.m. av. O <sub>2</sub> ) | 53  | 45 |    |
| Sodium hypochlorite (p.p.m. av. Cl <sub>2</sub> )     | 200 |    |    |
| Cetyltrimethylammonium chloride (p.p.m.)              | 240 |    |    |
| Eicosyltrimethylammonium chloride (p.p.m.)            | 62  |    |    |
| Sodium chloride (p.p.m.)                              | 118 |    |    |
| Copper sulfate (M <sup>2+</sup> × 10 <sup>-5</sup> )  | 1.2 |    |    |
| Initial solution pH                                   | 9.3 |    |    |

Bleaching of these solutions was then tested at various solution temperatures and performance recorded over periods of bleaching time. Results are summarized graphically in the drawing. The composition of the invention (No. 10) performs significantly better than monopersulfate alone (No. 13) and compares favorably with highly concentrated NaOCl (No. 11).

#### FABRIC SOFTENING TEST

Softening was tested under standard U.S. conditions of 125° F. wash (7 gr./gal. hardness) followed by 100° F. rinse with 7 gr./gal. hardness. Loads were washed in the automatic mini washer using 0.9 cup Tide, 1½ gallons of water and a 5½ pound load equivalent. The standard load contained 4 terry wash cloths. Compositions were tested for two cycles, and the terry cloths were graded by a panel of 5 expert judges using the method of round robin paired comparisons.

The softness of the fabrics treated with Composition No. 10 (Table II concentration) was judged to be significantly greater than the Tide control. Substantially similar results are obtained with Compositions Nos. 3 and 9.

What is claimed is:

1. A dry bleach and fabric-softening composition consisting essentially of:

- (A) from about 8% to about 60% by weight of a bleaching agent selected from the group consisting of
  - (1) sodium monopersulfate,
  - (2) potassium monopersulfate,
  - (3) an organic peroxyacid or water-soluble salt thereof, said peroxyacid having the general formula



wherein R is selected from the group consisting of alkylene groups containing from 1 to about 16 carbon atoms and arylene groups containing from 6 to about 8 carbon atoms and Y is a group providing an anionic moiety in aqueous solution, and

(4) mixtures thereof;

(B) from about 10% to about 60% by weight of a quaternary ammonium compound selected from the group consisting of



5

10

15

20

25

30

35

40

45

50

55

60

65

70

75

and



wherein R<sub>1</sub> is an alkyl group containing from about 12 to about 20 carbon atoms; R<sub>2</sub> is selected from the group consisting of alkyl groups containing from about 1 to 14 carbon atoms, cycloalkyl groups containing from about 5 to 8 carbon atoms, carboxymethyl groups, aryl groups containing from about 6 to 8 carbon atoms, alkaryl groups containing from about 7 to 10 carbon atoms, pyridyl, and groups of the general formula  $-(\text{C}_3\text{H}_6\text{O})_a(\text{C}_2\text{H}_4\text{O})_b\text{H}$  wherein a and b are integers and a+b is 1 to 50; R<sub>3</sub>, R<sub>4</sub> and R<sub>5</sub> are each selected from the group consisting of alkyl groups containing from about 1 to 3 carbon atoms, aryl groups containing from about 6 to 8 carbon atoms, cycloalkyl groups containing from about 5 to 8 carbon atoms, carboxymethyl groups, alkaryl groups containing from about 7 to 10 carbon atoms, pyridyl, and groups of the general formula



wherein a and b are integers and a+b is 1 to 50; R<sub>6</sub> has the definition of the R<sub>3</sub>, R<sub>4</sub> and R<sub>5</sub> groups or is H; R<sub>7</sub> is selected from the group consisting of alkylene groups containing 1 to 3 carbon atoms, arylene groups containing 5 to 8 carbon atoms and groups of the formula



wherein X is selected from the group consisting of chloride, fluoride, nitrate, sulfate, methylsulfate, carbonate, chlorate, hydrogen phosphate, dihydrogen phosphate and hydroxide; and wherein n is 1 when X is monovalent and n is 2 when X is divalent;

(C) from about 10% to about 75% by weight of a buffering agent effective to maintain a solution pH of from about 7 to about 10 when said composition is dissolved in water for bleaching; said composition containing sufficient chloride salt to provide from about 5 to about 100 grams of ionizable chlorine per kilogram of the total composition.

2. The composition of claim 1 wherein the bleaching agent is potassium monopersulfate.

3. A composition in accordance with claim 1 wherein the bleaching agent is selected from the group consisting of monoperazelaic acid and diperazelaic acid.

4. A composition in accordance with claim 1 which contains in addition from about 0.08% to about 8% by weight of a water-soluble salt of a transition metal element.

5. A composition in accordance with claim 1 which contains from about 2% to about 10% of a water-soluble alkali metal or alkaline earth metal chloride.

6. A composition in accordance with claim 1 wherein the quaternary ammonium compound is a mixture containing from about 2% to about 10% by weight of the total composition of an eicosyltrimethylammonium compound and about 8% to about 30% by weight of the total composition of a cetyltrimethyl- or octadecyltrimethylammonium compound.

7. A concentrated, dry bleach and fabric-softening composition consisting essentially of:

- (A) from about 8% to about 60% by weight of a bleaching agent selected from the group consisting of
  - (1) sodium monopersulfate,
  - (2) potassium monopersulfate,
  - (3) an organic peroxyacid or water-soluble salt

## 15

thereof, said peroxyacid having the general formula



wherein R is selected from the group consisting of alkylene groups containing from 1 to about 16 carbon atoms and arylene groups containing from 6 to about 8 carbon atoms and Y is a group providing an anionic moiety in aqueous solution, and

- (4) mixtures thereof;  
(B) from about 10% to about 60% by weight of a quaternary ammonium compound selected from the group consisting of



and



wherein  $\text{R}_1$  is an alkyl group containing from 12 to about 20 carbon atoms;  $\text{R}_2$  is selected from the group consisting of alkyl groups containing from about 1 to 14 carbon atoms, cycloalkyl groups containing from about 5 to 8 carbon atoms, carboxymethyl groups, aryl groups containing from about 6 to 8 carbon atoms, alkaryl groups containing from about 7 to 10 carbon atoms, pyridyl and groups of the general formula  $-(\text{C}_3\text{H}_6\text{O})_a(\text{C}_2\text{H}_4\text{O})_b\text{H}$  wherein  $a$  and  $b$  are integers and  $a+b$  is 1 to 50;  $\text{R}_3$ ,  $\text{R}_4$  and  $\text{R}_5$  are each selected from the group consisting of alkyl groups containing from about 1 to 3 carbon atoms, cycloalkyl groups containing from about 5 to 8 carbon atoms, carboxymethyl groups, aryl groups containing from about 6 to 8 carbon atoms, alkaryl groups containing from about 7 to 10 carbon atoms, pyridyl, and groups of the general formula



wherein  $a$  and  $b$  are integers and  $a+b$  is 1 to 50;  $\text{R}_6$  has the definition of the  $\text{R}_3$ ,  $\text{R}_4$  and  $\text{R}_5$  groups or is H;  $\text{R}_7$  is selected from the group consisting of alkylene groups containing 1 to 3 carbon atoms, arylene

## 16

groups containing 5 to 8 carbon atoms and groups of the formula



wherein X is selected from the group consisting of chloride, fluoride, nitrate, sulfate, methylsulfate, carbonate, chlorate, hydrogen phosphate, dihydrogen phosphate and hydroxide; and wherein  $n$  is 1 when X is monovalent and  $n$  is 2 when X is divalent;

- (C) from about 1% to 15% of a water-soluble alkali metal or alkaline earth chloride;  
(D) from about 0.08% to about 8% by weight of a water-soluble salt of a transition metal element; and  
(E) from about 10% to about 75% by weight of a buffering agent effective to maintain a solution pH of from about 7 to about 10 when said composition is dissolved in water for bleaching;

said composition containing sufficient chloride salt to provide from about 5 to about 100 grams of ionizable chlorine per kilogram of the total composition.

8. A composition in accordance with claim 7 wherein the bleaching agent is selected from the group consisting of diperoxazelaic acid, diperoxyisophthalic acid, diperoxyterephthalic acid, 4 - chlorodiperoxyphthalic acid, the monosodium salt of diperoxyterephthalic acid and a monoperoxy compound of the general formula



wherein R is an alkyl group of from about 8 to about 18 carbon atoms and wherein  $\text{X}^1$  and  $\text{Y}^1$  are each selected from the group of cations consisting of hydrogen, sodium, potassium, ammonium and substituted ammonium cations.

## References Cited

## UNITED STATES PATENTS

- 40 3,360,470 12/1967 Wixon ----- 252-99  
3,048,546 8/1962 Lake ----- 252-95  
3,353,902 11/1967 Diamond ----- 252-8.8

MAYER WEINBLATT, Primary Examiner

U.S. CL. X.R.

8-108, 111; 252-8.75, 8.8, 99

PO-1050  
(5/69)

UNITED STATES PATENT OFFICE  
CERTIFICATE OF CORRECTION

Patent No. 3,749,673 Dated July 31, 1973

Inventor(s) John Paul Jones and Charles H. Nicol

It is certified that error appears in the above-identified patent and that said Letters Patent are hereby corrected as shown below:

Column 4, line 47, delete "micslles" and insert therefor  
-- micelles --

Column 4, line 51, delete "virture" and insert therefor  
-- virtue --

Column 4, line 57, delete "chloride" and insert therefor  
-- chlorine --

Column 5, line 50, delete "aproximately" and insert therefor  
-- approximately --

Column 5, line 70, delete "othe" and insert therefor -- other --

Column 7, line 13, delete "hydrogen" and insert therefor  
-- dihydrogen --

Column 7, line 22, delete "[C<sub>20</sub>H<sub>39</sub>N(CH<sub>3</sub>)<sub>3</sub>]<sub>2</sub>HPO<sub>4</sub>" and insert therefor  
-- [C<sub>20</sub>H<sub>39</sub>N(CH<sub>3</sub>)<sub>3</sub>]<sub>2</sub>HPO<sub>4</sub> --

Column 7, line 53, delete "Conseqeuntly" and insert therefor  
-- Consequently --

Column 8, line 50, delete "Transistion" and insert therefor  
-- Transition --

Column 8, line 64, delete "necessaary" and insert therefor  
-- necessary --

Column 9, line 37, after "Test" replace the period with a comma.

Table I, after "Cetyltrimethylammonium" delete "choride" and  
insert therefor -- chloride --

PO-1050  
(5/69)

UNITED STATES PATENT OFFICE  
CERTIFICATE OF CORRECTION

Patent No. 3,749,673 Dated July 31, 1973  
Inventor(s) John Paul Jones and Charles H. Nicol Page - 2

It is certified that error appears in the above-identified patent  
and that said Letters Patent are hereby corrected as shown below:

Table II, after "Diperazelaic acid" delete " $O^2$ " and insert  
therefor --  $O_2$  --

Column 15, line 16, delete " $R_5$ " and insert therefor --  $R_4$  --

Signed and sealed this 1st day of January 1974.

(SEAL)  
Attest:

EDWARD M.FLETCHER,JR.  
Attesting Officer

RENE D. TEGTMEYER  
Acting Commissioner of Patents